

W. D. SNOW.  
FLOOR CLOTH.  
APPLICATION FILED JULY 27, 1915.

1,184,584.

Patented May 23, 1916.



Fig. 1.



Fig. 2.

Inventor.

William D. Snow.

# UNITED STATES' PATENT OFFICE.

WILLIAM D. SNOW, OF WINTHROP, MAINE.

## FLOOR-CLOTH.

1,184,584.

Specification of Letters Patent. Patented May 23, 1916.

Application filed July 27, 1915. Serial No. 42,119.

*To all whom it may concern:*

Be it known that I, WILLIAM D. SNOW, a citizen of the United States, residing at Winthrop, in the county of Kennebec and State of Maine, have invented certain Improvements in Floor-Cloths, of which the following is a specification.

My invention is a floor cloth comprising, in its preferred form, a body of sheeted paper or felt saturated with bitumen, a face printed to provide any desired design, and a back of woven material; and my leading object is to provide an inexpensive and ornamental product that is comparatively strong and durable, eliminating the tendency of usual floor coverings comprising tar paper and the like to rupture and tear.

The characteristic features of my improvements are more fully disclosed in the following description and the accompanying drawings in illustration thereof.

In the drawings, Figure 1 is a part sectional plan view of a piece of floor cloth embodying my improvements, and Fig. 2 is a section of the same.

My improved floor cloth, as illustrated in the drawings, comprises a body composed of a sheet of tar paper or felt saturated with bitumen 1, an ornamental face 2 produced by printing in oil paints upon a surface of the body 1, and the back 3 composed of a strengthening fabric such as muslin, duck or burlap, which is cemented to the body by any suitable adhesive, such as a coating of bitumen 4 applied to the tar paper and having the backing pressed thereon. This floor cloth, provided with an inexpensive body of considerable thickness and protected on both surfaces, has the advantages of comparative flexibility, comparative imperviousness to water and strength.

I have found that a body of the character described absorbs a certain percentage of bitumen or mineral pitch and inexpensive varnishes mixed with clay, which provide efficient binders of considerable body, the substance of which virtually becomes a part of the body and penetrates and fills the interstices of coarsely woven fabrics used as a backing, so that such backing is virtually incorporated in the outer stratum of the body, by which it is held so that it is practically undetachable and is also protected from deterioration due to the fact that its fibers are largely embedded.

Having described my invention, I claim:

1. A floor cloth comprising a body of sheeted fibrous material saturated with a bituminous substance, a coating on one surface thereof, and a strengthening fabric cemented on the opposite surface thereof.

2. A floor cloth comprising a sheet of tar paper, paint on one surface thereof, and a woven fabric cemented on the other surface thereof.

3. A floor cloth comprising a body of saturated felt, a coating of paint on a surface thereof, a coarsely woven fabric, and a cement adapted to penetrate said felt and fabric whereby said fabric is secured to said felt.

4. A floor cloth comprising a body of saturated felt having a coated face, a coarsely woven backing fabric, and a cement which penetrates through the meshes of said fabric and adheres to said body, whereby said fabric and body are fixed together.

In testimony whereof I have hereunto set my name this 20th day of July, 1915.

WILLIAM D. SNOW.